

July 20, 1926.

1,592,823

W. H. CROFT ET AL

CASTING METAL ALLOYS

Filed Jan. 2, 1925

2 Sheets-Sheet 1

Fig. 1.



Fig. 2.



Fig. 4.



Fig. 3.



Fig. 6.



Fig. 7.



Fig. 8.



William H. Croft  
Robert J. Schumacher  
Barney J. W. G. *Inventors*  
Attorneys

July 20, 1926.

W. H. CROFT ET AL

1,592,823

CASTING METAL ALLOYS

Filed Jan. 2, 1925

2 Sheets-Sheet 2

59

Fig. 10.



60 59 61

Fig. 11.



Fig. 13.



William H. Croft  
Robert J. Sturmacher  
Barney J. Wilson  
Attorneys

Patented July 20, 1926.

## UNITED STATES PATENT OFFICE.

WILLIAM H. CROFT AND ROBERT J. SHOEMAKER, OF CHICAGO, ILLINOIS.

## CASTING METAL ALLOYS.

Application filed January 2, 1925. Serial No. 198.

Our invention relates to the production, by casting, of alloys or mixtures of metals which have a tendency to become segregated or disassociated when cooling in the mold, such, for example, as copper and lead used in the manufacture of bearings, anti-friction bushings, packing rings, and the like, and one of the primary objects of the invention is to provide a novel method of casting articles of this sort whereby the character of the same is improved, particularly for anti-friction purposes, by making the alloy more uniform and homogeneous, through prevention of segregation and by more complete freedom from abrasive impurities and from gas bubbles and other imperfections.

A further object is to provide certain novel apparatuses for carrying out the improved method.

20 A further object is to provide, as a new article of manufacture, anti-friction metal castings having the hereinafter described advantageous characteristics.

The invention is illustrated in the accompanying drawings, wherein—

Fig. 1 is a sectional perspective view of the metallic mold forming part of a molding apparatus for the manufacture of locomotive piston rod packing rings.

30 Fig. 2 is a view, in perspective, of the sand cope of this apparatus.

Fig. 3 is a similar view of the metallic core.

Fig. 4 is a vertical sectional view of the molding apparatus, the separate parts of which are shown in Figs. 1, 2 and 3, with said parts in assembled relation and the metal poured.

Fig. 5 is a sectional perspective of the 40 packing ring cast in the apparatus shown in Figs. 1 to 4 inclusive before the sprues have been removed.

Fig. 6 is a view, in sectional perspective, of the metallic mold element of another form of apparatus for casting packing rings or the like.

Fig. 7 is a vertical sectional view of the assembled apparatus with the metal poured.

Fig. 8 is a sectional perspective of the 50 packing ring casting in the apparatus of Figs. 6 and 7 before the sprue has been removed.

Fig. 9 is a view, in perspective, of a metallic mold element for apparatus for casting cylindrical bushings.

Fig. 10 is a sectional perspective of the cope for this apparatus.

Fig. 11 is a vertical sectional view of the assembled apparatus.

Fig. 12 is a sectional perspective of the 60 base member of the apparatus, and

Fig. 13 is a plan view of the collapsible metal core forming part of the apparatus of Figs. 9 to 12.

For packing the piston rods of steam engines operated by superheated steam, it has been found necessary to provide packing rings which will stand higher temperatures than the babbitt customarily used with engines operated by saturated steam.

The packing rings should be made of anti-friction metal or metals and an alloy of copper and lead has been found suitable for the purpose except that when the rings are cast in sand molds the cooling is so slow that there is a tendency for the metals to become segregated or disassociated, the reason being, probably, that fused copper and lead form a physical mixture rather than an alloy in the strict sense of the word. Moreover, the sand is likely to be washed into the casting forming slag, undesirable because of its abrasive character, and gas holes in the casting.

We have found that while it is not practical (at least in the manufacture of cored castings) to use an all metal mold, for reasons which will appear, it is possible to effectually prevent the segregation of the ingredient metals by using a composite mold comprising metal mold and core elements between which the mold cavity is formed, and cope in which the pouring gates are arranged which is formed of molder's sand. When the fused metal mixture reaches the mold cavity it cools so rapidly that disassociation of the ingredient metals is prevented. At the same time there is considerable shrinkage, but to provide metal to fill the cavity when this shrinkage takes place, the pouring gate or gates are filled or partially filled during the pouring operation and as this excess metal in the gates is in contact with sand, it cools much more slowly than the metal in the mold cavity, and will remain sufficiently fluent so as to flow down into the mold cavity to make up for shrinkage. If the cope were of metal the pouring gate would be likely to freeze so as to make this operation impossible. While the

amount of metal necessary for making up for shrinkage may be small the volume in the gates should be large enough to insure against too rapid cooling. If an all-metal 5 mold is employed it will be necessary to maintain the fluidity of the metal in the pouring gates by some other means, for example, by pressure as in die casting. In order to prevent adherence of the casting to 10 the metallic core it is desirable, and in most cases necessary, to remove the core from the casting while the latter is hot, that is, before it has shrunk on the core. We find it desirable to remove the core while the casting 15 is at red heat, if the casting is of bronze composition, that is, at approximately 1000° to 1200° Fahrenheit; but for a copper-lead mixture the metal should be allowed to cool more than this, for instance, to about 600° 20 Fahrenheit in order that the lead may not sweat out. The casting in either case is allowed to remain in the mold until it has finally set.

Referring to Figs. 1 to 5 inclusive, 25 designates an annular cast iron mold element formed, preferably, with a tapered opening 26 and recessed at 27 to provide, with the cast iron core 28, a cavity to receive the molten metal. This cavity, in the 30 form of the apparatus shown in Figs. 1 to 4, converges downwardly as indicated at 29, the conical surface, however, not extending quite to the inner edge of the mold element so that this edge of the packing ring, indicated at 30, is blunt as shown at 31. The core 28 is tapered to fit the tapered opening 26 in member 25 and in assembling the parts the upper edge of the core is flush with the upper edge of element 25. The 35 mold cavity is covered by a green sand cope 32 formed with a pouring opening and a riser designated 33 and 34. The metal poured into the mold cavity through one of these openings will, of course, rise in the other to the extent of excess of metal over that necessary to fill the cavity. The metal in the cavity chills rapidly and shrinks. The metal in openings 33, 34 cools much more slowly so that it will remain fluent and will 40 flow into the cavity to make up for the shrinkage of the metal therein. As soon as the metal has hardened but before it has taken its final set, the cope is removed and the metal core is knocked out. When the casting has set it is removed from the mold element 25, after which the sprues 35, 36 are cut off and the surfaces of the ring finished as may be necessary. We have found that there is little or no washing of the sand 45 from the cope into the casting. The intermingling of sand with metal took place, with the old method of sand molding, largely when the hot metal struck the sand bottom of the mold cavity. The sand cope permits 50 the ready escape of gases from the mold cavity. If desired the casting may be gated tangentially so as to minimize gassing due to direct impingement of the molten metal against the wall of the mold.

The preferred ingredients for a packing 70 ring to be used as indicated, are as follows: 35% to 40% copper, 3% to 5% nickel, the balance lead. The nickel gives a more intimate amalgamation of the other metals. Preferably we use a flux consisting of phosphor copper (85% copper and 15% phosphorous). This flux is used in quantities of 75 from 1 to 4 ounces per 100 pounds of metal. It acts as a dioxidizer so that the metal flows more freely.

The same method may be used for casting any unstable mixture of metals, such, for example, as a mixture of 68% copper, 25% 80 lead and 7% tin.

In Figs. 6, 7 and 8 we have illustrated a 85 modified, and in some respects more desirable method of casting the same sort of packing ring or other like article. In this apparatus the cast iron mold element 37 is arranged, in a position inverted with respect to that of element 25, upon an iron base plate 38. The metallic core 39 is annular in form but externally tapered as is core 28. Within the metal core 39 is a dry sand core 40 which is formed with a pouring gate 41 and projects up through the green sand cope 42. An orifice 43 through the sand and metal cores leads to the mold cavity 44. The mold element 37 is formed with a plurality of gas orifices 45 to allow escape of gas from the mold cavity into the green sand of the cope. This form of casting apparatus has the advantage that the wide end 45 of the packing ring 47 (Fig. 8) has a relatively smooth surface requiring but little finishing. Whatever slag there may be in the metal collects in the tapered end of the ring from which it may be removed by a simplified machining operation. When the casting has sufficiently set the cope 42 is removed and the mold 37, core 39 and the casting are inverted and the core knocked out of the mold element 37 from which the casting may then be removed and its sprue 48 cut off.

In Figs. 10 to 12, I have shown apparatus for casting the cylindrical bushing designated 49. A suitable alloy for an anti-friction bushing of this sort consists of 70% copper, 5% tin and 25% lead. These 90 metals tend to segregate when cast in sand. The molding apparatus comprises separable metallic mold members 51, 52 adapted to be secured together by bolts 53, a metal base plate 54 formed with a circular recess 55, a collapsible metal core 56, 57, 58, preferably tapered, the lower end of which is adapted to fit the recess 55, and a sand cope 59 formed with pouring gate and riser 60 and 61 adapted to align with the mold cavity 95 100 105 110 115 120 125 130

ity between mold elements 51, 52 and the core. The core is made preferably in three parts 56, 57, 58, as shown in Fig. 13; part 58 being a wedge which can be readily knocked out when the core is to be removed. For this purpose the core sections are formed with recesses 62 for a chisel. The core is removed while the casting is hot. After the casting is set it may be removed from the mold. The embodiment of the invention disclosed in Figs. 10 to 12 is not claimed in its specific details in this application as it forms part of the subject matter of an application by us, Serial No. 111,993, filed May 27, 1926 as a continuation in part of this application.

It will be understood that the apparatuses and methods described are, so far as details are concerned, merely illustrative of the principles of our invention which we propose to claim as broadly as the state of the art will warrant.

We claim:

1. Molding apparatus for casting metal

alloys of the character described, comprising, in combination, a metallic mold element having a tapered opening therein, a tapered metallic core to fit into said opening, and a sand element formed with a pouring gate leading to the cavity between said mold element and core.

2. Molding apparatus for casting metal alloys of the character described, comprising, in combination, an annular metallic mold element, the opening through which is tapered, a tapered metallic core to fit into said opening, and a sand cope provided with a pouring gate leading to the mold cavity.

3. Molding apparatus for casting metal alloys of the character described, comprising, in combination, an annular metallic mold element having an opening therethrough, a metallic core to fit into said opening, and a sand cope provided with a pouring gate leading to the mold cavity.

WILLIAM H. CROFT.  
ROBERT J. SHOEMAKER.